# EUROPEAN PATENT SPECIFICATION

(11) **EP 0 028 653 B1**
(45) Date of publication and mention of the grant of the patent: **04.07.1984**
(21) Application number: 80900071.4
(22) Date of filing: 19.12.1979
(51) Int. Cl.: B22D 29/00, B22D 13/10

(54) **TUBULAR CAST PIECE INNER SURFACE WORKING APPARATUS**
VORRICHTUNG FÜR DIE MASCHINELLE BEARBEITUNG DER INNENWAND EINES GEGOSSENEN, ROHRFÖRMIGEN WERKSTÜCKS
DISPOSITIF POUR L'AJUSTAGE DE LA SURFACE INTERNE D'UN ARTICLE TUBULAIRE MOULE

(30) Priority: 19.12.1978 JP 158927/78
(43) Date of publication of application: 20.05.1981
(73) Proprietor: KUBOTA LIMITED, Osaka-shi Osaka 556 (JP)
(72) Inventor: TAKESHITA, Kimio, Fujiidera-shi, Osaka 583 (JP); MIYAGAKI, Moriyuki, Minamikawachi-gun Osaka 589 (JP); AMAKASU, Toshinari, Nara-shi Nara 630 (JP); UGATA, Ken, Nara-shi Nara 631 (JP); NAKAISHI, Masao, Takaishi-shi Osaka 592 (JP)
(74) Representative: Cabinet HERRBURGER
(86) International application number: JP7900319
(87) International publication number: WO8001257

## Description

### Technical Field

This invention relates to a tubular cast piece apparatus of pressure-compacting the tubular cast piece inner surface in a predetermined temperature range.

### Background Art

Tubular cast pieces are manufactured generally by centrifugal casting method or by casting method employing core means. With such method, it is known that there appear shrinkage cavities or pores on the tubular inner surface as the tubular cast piece cools down. Consequently, it is clear that such shrinkage cavities or pores lower the strength and gastightness of the tubular cast pieces.

In order to eliminate the drawbacks mentioned above, there has conventionally been proposed the method, in manufacturing the tubular cast pieces by centrifugal casting method, of pouring melt into the metal mold for centrifugal casting and pressing the tubular inner surface employing rollers or the like prior to completion of solidification of the melt, to thereby pressure-sealing the shrinkage cavities or pores.

In case of using the tubular cast pieces as fluid pipe-line and the like, it has on the other hand been required to manufacture the products such that the strength and gastightness of the pipes themselves are excellent in the matter of course and that the products have the pipe inner surface excellent in abrasion resistance and corrosion resistance and at the same time low in fluid resistance as is realized by enhancing the hardness of the pipe inner face.

However, with the conventional methods for pressure-demolishing and sealing and shrinkage cavities or pores it may all right have been possible to crush down the shrinkage cavities or pores but it has not been possible to harden the tubular inner surface, since thereby one gives pressure on the tubular inner surface in its soft state prior to completion of the melt solidification.

On the other hand, practiced generally and widely with the intension of hardening the cast piece surface is a method of pressure-working the surface at normal temperature, namely of applying the so- called cold working. However, an apparatus is required to generate tremendous heavy pressure when to crush down at the same time the shrinkage cavities or pores with such a method, and there is a drawback such as causing distortion in the tubular body by applying such heavy pressure, and so such a method has not actually been practiced.

From the specification DE-C-750 924 is already known an art of centrifugal casting, according to the precharacterising part of claim 1.

However the art is not aware of the transition temperature that affects material properties of a tube casted and pressed by rollers such as hardness, flexibility and tensile strength.

### Disclosure of Invention

In view of the limitation of the prior art as mentioned above, this invention has as its object to provide a tubular cast piece inner surface working apparatus which is adapted to position a pressing head of pressing means in inner hollow space of a tubular cast piece formed by casting; and also adapted to cause said pressing head to pressure-compact the said tubular cast piece inner surface within a temperature range starting from that immediately after completion of the said tubular cast piece solidification to the transition temperature, while bringing the said pressing head and the said tubular cast piece in relative rotation.

Such an apparatus is designed to be suited for utilizing the mechanical properties of metals in general, especially the "elongation" thereof. It will facilitate the working remarkably when the temperature is maintained above the transition temperature. Experiments have confirmed a fact that by pressure-compacting the metal surface while bringing the metal and the pressing element in relative rotation, even immediately after the metal solidification, hardness of the worked surface is advantageously enhanced. The transition temperature means the temperature where the mechanical properties (tensile strength and elongation) show abrupt changes.

The apparatus according to this invention is therefore constructed to have a structure adapted both to pressure-seal the shrinkage cavities or pores and to harden the surface of the tubular cast piece, the sealing and the hardening being executed at a single stroke of the head.

It will now be made possible to heighten and equalize metal structure density near the tubular cast piece inner surface, thus expecting enhancement of the strength and gastightness of the overall tubular cast piece, and simultaneously to harden the inner surface so as to make the tubular cast piece excellent in abrasion resistance and corrosion resistance and at the same time low in resistance in fluid transfer.

It can therefore be rightly said that quite remarkable industrial value accrues therefrom in manufacturing the various tubular cast pieces, for instance as hydraulic cylinder parts, internal combustion engine cylinder parts, various kinds of cast iron pipes, vacuum vessel parts and various rolls, atomic power station piping and the like or else high-strength aluminium alloy casting, cast steel pipes and the like.

The object of this invention is therefore to provide a tubular cast piece inner surface working apparatus comprising a pressing head which is operatively connected to a travel causing device, the apparatus further comprising a driving means for driving a metal mold for centrifugal casting.

For attaining such an object, the invention provides a tubular cast piece inner surface working apparatus having a pressing head which is operatively connected to a travel causing device and driving means for driving a metal mold for centrifugal casting (DE-C-750 924) characterized in that it comprises a plurality of pressing rollers arranged about the pressing head at equal intervals and cam means for shifting the pressing rollers in the radial direction of the tubular cast piece to press the inner surface of the tubular cast piece, said cam means including an oil hydraulic cylinder having a piston rod provided with taper cam means (cam surfaces) at one end thereof, and a plurality of supporter members for idly supporting the three pressing rollers respectively on each of supporting shafts mounted thereof and each having a cam surface substantially contacting with the taper cam means (cam surfaces) of the piston rod.

The invented apparatus is advantageous, in comparison with the apparatus shown in DE-C-750924, in that the pressing power generating unit is movable in unison together with the pressing head which has plural pressing rollers rotatable more easily about their own axes. Therefore, the pressure applied to a workpiece can be very easily maintained constant during the axial movement of said pressing head.

Further objects and advantages of this invention will become clear from the explanation now to follow.

### Brief Description of Drawings

Drawings show, by way of example, the best embodiment of the tubular cast piece inner surface working apparatus according to this invention, wherein:
Fig. 1 is a vertical section of an essential portion of a centrifugal casting machine with rough overall side elevation of a tubular cast piece inner surface working apparatus,
Fig. 2 is an enlarged end view of pressing means as viewed according to arrows II-II in Fig. 1,
Fig. 3 is an enlarged side elevation, partly in section, of an essential portion of pressing means,
Fig. 4 is a photographic picture of an aluminium alloy tubular cast piece section showing the states of said piece before and after the inner surface working executed by means of the invented apparatus,
Fig. 5 is a vertical sectional view showing a tubular cast piece which has a round section and is to be worked by means of the apparatus,
Fig. 6 is an end view of the tubular cast piece shown in Fig. 5, and
Fig. 7 is a vertical sectional view showing a tubular cast piece which has a tapered outer surface and is also to be worked by means of the apparatus.

### Best Mode for Carrying Out the Invention

This invention is now explained in more detail hereunder with reference to the accompanying drawings.

Fig. 1 shows a vertical section of an essential portion of a centrifugal casting machine with rough overall side elevation of a tubular cast piece inner surface working apparatus. The invention will be utilized so as to centrifugally cast and form the tubular cast piece, but the piece be formed same by any other manner. Shown at (1) is a metal mold for centrifugal casting, and at (2) is a tubular cast piece which is formed in the said metal mold (1). The tubular cast piece (2) is equipped at an end portion, as is illustrated, with a flange (2a). The numeral (3) are indicating plural driving rollers which support the said metal mold (1) and also drive same into rotation. These driving rollers (3) are connected to an electric motor (4) via suitable means, both of these members together with the said metal mold (1) constituting driving means (5).

Indicated at (6) is pressing means, and it is constructed with: a pressing head (6a) to be inserted and positioned in inner hollow space of the said tubular cast piece (2); a pressing power generating unit (6b) adapted to generate the pressing power of the pressing head (6a); and a travel-causing device (6c) to move the pressing power generating unit (6b) together with the pressing head (6a) along the axial direction of the said tubular cast piece (2).

The said travel-causing device (6c) comprises an oil hydraulic cylinder (19) fixed in a stationary position, and a well-known oil hydraulic pump system (not illustrated) adapted to supply oil pressure thereto. A piston rod (20) of the said oil hydraulic cylinder (19) is connected to the said pressing power generating unit (6b).

The pressing power generating unit (6b) comprises a holder (10) to sustain the said pressing head (6a), an oil hydraulic cylinder (9), a piston rod (11) thereof (see Fig. 3) and an oil hydraulic pump system (not illustrated) driving the oil hydraulic cylinder (9). The pressing power generating unit (6b) is movable to travel on rail means (7) so that said pressing head (6a) can be driven smoothly in the axial direction of the said tubular cast piece (2) by actuation of the said travel-causing device (6c).

The said holder (10) is adapted to extend out from the machine frame of said pressing power generating unit (6b) thereby sustaining the said pressing head (6a). The said piston rod (11) extends to pass through the inside of the said holder (10) for free advance towards the said pressing head (6a) for retraction therefrom. On the tip end of said rod there is formed a taper portion (11a). Indicated at (12) are three pressing rollers disposed at equal intervals in the circumferential direction of the said pressing head (6a), each of them having the rotary axis in parallel with the axis of the said piston rod (11).

In Fig. 3, an interval between the two pressing rollers is shortened for easier drawing and for clearer view.

Indicated at (18) is a guide member, with one end thereof fixed to the tip end of the said pressing head (6a) by means of a nut and with the other end thereof inserted into a hole bored in the said taper portion (11 a), and it functions as a guide when the taper portion (11 a) is operated to advance or retire.

The said pressing rollers (12) are mounted to be idly rotatable on supporting shafts (14) fixed on the respective supporter members (13). Each of the supporter members (13) is held to be slidable in the radial direction on the said piston rod (11) or the said tubular cast piece (2) relative to the said pressing head (6a) and has a cam surface (13a) formed on the side of the axis thereof. It is noted here that by the movement of the said piston rod (11) the taper portion (11 a) thereof comes to abut against the said cam surfaces (13a), thus to urge and push the said supporter members (13) and to cause the pressing rollers (12) provided thereon to urge and push against the inner surface of the said tubular cast piece (2). Thus, cam means (15) is constructed with the taper portion (11 a) of the piston rod (11) and the cam surface (13a) of the said supporter member (13). The said pressing roller (12) is constructed in a shape having a plain surface (12a) of narrow width in the central portion thereof and, on both sides thereof, slant surfaces (12b). By the use of the said flat surface (12a) of narrow width, the apparatus is advantageous in that it heighten the urging pressure force against the inner surface of the said tubular cast piece (2) so as to make smooth the inner surface. However, the pressing rollers may be of a bear- barrel shape of smooth gradual bulging, those having various shapes of bulging, or else cylindrical body and the like. The pressing rollers may be forced into rotation. Indicated at (16) are compression springs which are interposed between the said pressing head (6a) and the said supporter members (13) so that said springs compress the said supporter members (13) when same are urged and pressed by the action of said cam means (15). The compression springs (16) cause the said supporter members (13) to restore to the original positions, namely to the non-compaction-acting position, when the cam action has been released. Fig. 3 shows such state that the cam action by said cam means (15) has been released, thus with the compressing springs (16) extended and with the supporter members (13) in the non-compaction-acting position.

Indicated at (17), as shown in Figs. 1 and 2, is a cutting tool for scraping off the inner surface of the said tubular cast piece (2) and is mounted at the tip end of the said pressing head (6a).

Fig. 3 is drawn in such state that this cutting tool (17) has been removed.

Now, the apparatus of this invention is explained hereunder using the metal mold (1) for centrifugal casting as well as driving means (6) as mentioned above.

First, aluminium alloy melt is poured into the metal mold (1) for centrifugally casting the tubular cast piece (2). Subsequently, the pressing head (6a) of pressing means (6) is inserted and positioned in the inner hollow space of the tubular cast piece (2).

Immediately after completion of the said tubular cast piece (2) solidification, the oil hydraulic cylinder (9) of the pressing power generating unit (6b) is actuated, thus the piston rod (11) thereof is drawn and the taper portion (11 a) at the tip end thereof causes the supporter members (13) of the pressing rollers (12) to move towards the inner surface of the said tubular cast piece (12).

Each of the pressing rollers (12) functions thereby for pressure-compacting the inner surface of tubular cast piece (2).

During the above operations the said metal mold (1) is continuously rotated and the said pressing rollers (12) are made to effect the pressure compacting while idly rotating.

On the other hand, the said pressing power generating unit (6b) is then moved on rail means (7) by the travel-causing device (6c) so as to drive the said pressing head (6a) to travel in the axial direction of the tubular cast piece (2) thereby effecting the pressure compacting over the whole tubular inner surface.

If a scraping-off stage is executed prior to the said pressure-compacting stage. the inner diameter of the tubular cast piece (2) will be made more uniform thus enabling a more effective urging pressure force by means of the pressing rollers (12) all over the tubular cast piece (2).

The tubular cast piece of more excellent quality will be obtained in such case.

Inversely, if the scraping-off stage is executed after the said pressure-compacting stage any desired inner diameter of the tubular cast piece (2) will be attained.

Furthermore, by first effecting the scraping-off stage and subsequently performing the inner surface pressure-compacting stage and thereafter performing once again the scraping-off stage, both of the advantages of the said two manners will be achieved.

It is still further possible to obtain the tubular cast pieces of the qualities as are suited for the various uses, by supplementing a stage of applying certain special surface hardening treatment or the like after the final scraping-off stage is over.

Now, this invention mentioned above is explained hereunder with reference to Field Example 1:

### Field Example 1

One took AI - 4.5%Mg alloy, cast same by metal mold centrifugal casting so a wall thickness of 35 mm, kept the tubular cast piece at 300°C after completion of the solidification, retaining same as integral with the casting mold, and put the inner surface thereof to a pressure by the pressing rollers at the urging pressure force of 200 kg/cm², and caused same to make two reciprocations over the full length on the inner surface, thus to cause reduction of 0.5 mm in the cast wall thickness.

A photographic picture taken of the section of the thusly obtained tubular cast piece, after applying dyeing color penetration flaw detection thereon, is Fig. 4. Central portion of the tubular cast piece of Fig. 4 is the portion the pressure-compacting mentioned above has been applied on, while both lateral sides thereof are left in the state just as centrifugally formed.

As is clear from Fig. 4, it can be recognized that the portion on which the inner surface working has been applied by use of the apparatus of this invention appears to be white, namely that it has been changed to have dense structure, while both lateral sides thereof appear to be black (-actually, they are dyed in red color-) on account of shrinkage cavities or pores as generated.

Shown in Table 1 are differences between mechanical properties of the inner diameter periphery portion of cast pieces manufactured by the invented apparatus and the known apparatus:

Wherein these result are with respect to each test piece cut out in size of 14 mm outer diameter with its center located at 10 mm from the inner diameter periphery of the tubular cast piece.

Next, Field Example 2 for demonstrating the surface hardening ensuing on pressure-compacting the tubular cast piece inner surface as is the object of this invention, is now described hereunder:

### Field Example 2

Shown in Table 2 are temperatures during the pressure-compacting after casting the tubular cast pieces using aluminium alloy substantially the same as in the said Field Example 1 with the pressure-compacting with urging pressure force of the pressing rollers set at 400 kg/cm², with showing of the relation with the hardness, at room temperature, of the inner surface and the unworked outer surface of the tubular cast piece as pressure-compacted at such temperature, as well as of the relation with the elongation and the tensile strength of the said aluminium alloy at such temperature of effecting the pressure-compacting:

As is clear from Table 2 above, it is seen that the inner surface hardness of the tubular cast piece on which the inner surface pressure working is effected at 500°C is greater than the unworked tubular cast piece outer surface hardness. It is further seen that the inner surface hardness gets increased as the pressure-compacting work temperature lowers, to approximately reach the limit at about 150°C-100°C.

On the contrary, it is seen that the elongation, as a mechanical property, of the said aluminium alloy shows remarkable increase as the temperature goes up higher, with a clear border line of about 100°C, namely the transition temperature.

From this, it is understood that by using the invented apparatus in the range from the temperature immediately after completion of the casting object metal solidification to the transition temperature of that metal it is then possible to crush down with mild pressure force the shrinkage cavities or pores at the state of mild steel property of that metal, thus enabling to obtain the metal structure dense in the wall thickness direction of the tubular cast piece and uniform approximately, and at the same time to enhance the worked surface hardness.

Since it is further noted from the said Table 2 that the tensile strength shows remarkable lowering as the temperature goes up higher with a clear border line of about 200°C, it is seen that when one practices the pressure-compacting work further preferably in the range from 450°C to about 200°C it is then possible to perform the inner surface compacting work to provide comparatively high value of hardness with milder pressure force.

By the way, showing in regard to the transition temperatures of other metals is, by way of example, 500°C with respect to steel and cast iron, 600°C with respect to 18-8 stainless steel and 450°C with respect to a copper alloy (70% copper, 30% zinc). As described above in detail, it is made possible according to this invention to work the tubular cast piece inner surface and to enhance the quality thereof, and it is further noted that by enlarging partially the pressure force at the earlier stage of the pressure-compacting work, namely at high temperature state, it is possible even to work out the pressure compacting for causing the stepped profile in the tubular inner surface, as shown in Fig. 5.

It should further be noted that the apparatus can also be applied on tubular cast pieces having tapered section as shown in Fig. 7 and on tubular cast pieces of polygonal outer shape as shown in Fig. 6.

By the way, though it has been made to construct pressing means (6) in this invention using oil hydraulic pressure, but such may as well be any construction only if the construction can press the tubular cast piece (2) inner surface.

Furthermore, with respect to the relative rotation the tubular cast piece (2) and the pressing head (6a) of pressing means (6) it is as well possible, even in the same case of using the metal mold for centrifugal casting machine, as mentioned above, to cause the side of the pressing head (6a) to rotate or to cause same and the metal mold (1) supporting the tubular cast piece (2) to rotate in directions opposite to each other.

Still further, it is also possible to make both of the said two in one and the same direction but with different circumferential speeds of both of them at the abutment portions.

Such manners for the relative rotation may be all the same also in case that one casts the tubular cast piece by using other casting manner and performs the pressure-compacting while sustaining the cast piece by any other chuck means or the like, and on the other hand it is also possible to use any suitable construction as driving means (5) to cause pressing means (6) and the tubular cast piece in the relative rotation.

### Industrial Applicability

As is clear from the above description, the tubular cast piece inner surface working apparatus thereof according to this invention may be utilized for the various uses since strength and gastightness of the tubular cast piece as well as abrasion resistance and corrosion resistance of the inner surface thereof can thereby be enhanced, thus to the tremendous advantage in the industrial application thereof.

## Claims

1. Tubular cast piece inner surface working apparatus having a pressing head (6a) which is operatively connected to a travel causing device (6c) and driving means (5) for driving a metal mold (1) for centrifugal casting characterized in that it comprises a plurality of pressing rollers (12) arranged about the pressing head (6a) at equal intervals and cam means (1 5) for shifting the pressing rollers (12) in the radial direction of the tubular cast piece to press the inner surface of the tubular cast piece, said cam means (15) including an oil hydraulic cylinder (9) having a piston rod (11) provided with taper cam means (cam surfaces) (11a) at one end thereof, and a plurality of supporter member (13) for idly supporting the three pressing rollers (12) respectively on each of supporting shafts (14) mounted thereon and each having a cam surface (13a) substantially contacting with the taper cam means (cam surfaces) (11a) of the piston rod (11).

2. Apparatus recited in claim 1, further comprising at least a compressing spring (16) disposed between each of the supporting members (13) and the pressing head (6a) for returning each of the pressing rollers (12) to its normal position when the oil hydraulic cylinder (9) is in non-operating position.

3. Apparatus recited in claim 2, wherein said pressing rollers (12) and said supporting member (13) are respectively three.

4. Apparatus recited in claim 3, the tubular cast piece inner surface working apparatus characterized in that with respect to the said pressing roller (12) there are formed: a plain surface (12a) in the central portion thereof; and on both sides of the surface, slant surfaces (12b).

5. Apparatus recited in claim 4, wherein said travel-causing device (6c) comprises an oil hydraulic cylinder (19) and a piston rod (20) which is connected to the pressing head (6a).

## Patentansprüche

1. Vorrichtung zur Bearbeitung der Innenfläche von Gußrohren mit einem mit einer Vorschubeinrichtung (6c) verbundenen Preßkopf (6a) und mit einer Antriebsvorrichtung (5) zum Antrieb einer Metallform (1) zum Zentrifugalgießen, gekennzeichnet durch mehrere, in gleichen Abständen am Umfang des Preßkopfes (6a) angeordnet Preßwalzen (12) und eine die Preßwalzen (12) in radialer Richtung des Gußrohres verschiebende Keilspanneinrichtung (15) zum Zusammenpressen der Innenfläche des Gußrohres, wobei die Keilspannvorrichtung (15) einen Ölhydraulikzylinder (9) enthält, der eine Kolbenstange (11) aufweist, die an einem Ende mit einer sich keilförmig verjüngenden Einrichtung bzw. einer im Querschnitt keilförmigen Oberfläche (11 a) versehen ist und mehrere Auflager (13) enthält, die die drei Preßwalzen (12) über an den Preßwalzen (12) befestigten Lagerwellen (14) abstützen und die jeweils eine im Querschnitt keilförmige Oberfläche (13a) aufweisen, die mit der sich verjüngenden, im Querschnitt keilförmigen Oberfläche (11 a) der Kolbenstange (11) in Berührung stehen.

2. Vorrichtung nach Anspruch 1, dadurch gekennzeichnet, daß mindestens eine Druckfeder (16) zwischen jedem der Auflager (13) und dem Preßkopf (6a) vorgesehen ist und die Preßwalzen (12) in die Normalstellung bewegt, wenn der Ölhydraulikzylinder (9) sich in der Ruhestellung befindet.

3. Vorrichtung nach Anspruch 2, dadurch gekennzeichnet, daß jeweils drei Preßwalzen (12) und Auflager (13) vorgesehen sind.

4. Vorrichtung nach Anspruch 3, bei der die Vorrichtung zur Bearbeitung der Innenfläche von Gußrohren dadurch gekennzeichnet ist, daß die Preßwalzen (12) im mittleren Abschnitt eine ebene und glatte Oberfläche (12a) und zu beiden Seiten der Oberfläch abgeschrägte Flächen (12b) aufweisen.

5. Vorrichtung nach Anspruch 4, dadurch gekennzeichnet, daß die Vorschubeinrichtung (6c) einen Ölhydraulikzylinder (19) und eine Kolbenstange (20) aufweist, die mit dem Preßkopf (6a) verbunden ist.

## Revendications

1. Dispositif pour le traitement de la surface intérieure d'une pièce tubulaire moulée comprenant une tête de compression (6a) associée en fonctionnement à un dispositif d'entraînement (6c), et des moyens moteurs (5) destinés à entraîner un moule métallique (1) de moulage centrifuge, dispositif caractérisé en ce qu'il comprend un certain nombre de rouleaux de pression (12) disposés à intervalles égaux autour de la tête de compression (6a), et des moyens de came (15) destinés à déplacer les rouleaux de pression (12) dans la direction radiale de la pièce tubulaire moulée pour comprimer la surface interne de cette pièce tubulaire moulée, ces moyens de came (15) comprenant un cylindre hydraulique (à huile (9) muni d'une tige de piston (11) équipée de moyens de came en biseau (surfaces de came) (11a) à l'une de ses extrémités, et un certain nombre d'éléments de support (13) destinés à supporter, en roue libre, les trois rouleaux de pression respectifs (12) de chacun des arbres de support (14) montés sur ceux-ci, et comportant chacun une surface de came (13a) venant directement en contact avec les moyens de came en biseau (surfaces de came) (11 a) de la tige de piston (11).

2. Dispositif selon la revendication 1, caractérisé en ce qu'il comprend, en outre, au moins un ressort de compression (16) disposé entre chacun des éléments de support (13) et la tête de compression (6a), pour ramener chacun des rouleaux de pression (12) dans sa position normale lorsque le cylindre hydraulique à huile (9) est en position inactive.

3. Dispositif selon la revendication 2, caractérisé en ce que les rouleaux de pression (12) et l'élément de support (13) sont respectivement au nombre de trois.

4. Dispositif selon la revendication 3, pour le traitement de la surface intérieure d'une pièce tubulaire moulée, dispositif caractérisé en ce que, pour ce qui concerne le rouleau de pression (12), on forme une surface plate (12a) dans sa partie centrale et des surfaces inclinées (12b) de part et d'autre de sa partie centrale.

5. Dispositif selon la revendication 4, caractérisé en ce que le dispositif d'entraînement (6c) comprend un cylindre hydraulique à huile (19) et une tige de piston (20) reliée à la tète de compression (6a).
